

Aug. 3, 1937.

E. HUBERT ET AL

2,088,858

MANUFACTURE OF ARTIFICIAL THREADS

Filed April 30, 1935

3 Sheets-Sheet 1

Fig. 2



Fig. 1



Fig. 1a



Inventors:

Emil Hubert,

Klaus Dammenberg,

Potter, Pierce & Scheffler.

By Attorneys

Aug. 3, 1937.

E. HUBERT ET AL

2,088,858

MANUFACTURE OF ARTIFICIAL THREADS

Filed April 30, 1935

3 Sheets-Sheet 2

Fig. 3



Fig. 4



Inventors:  
Emil Hubert,  
Lars Dammenberg,  
Potter, Pierce & Schaffler.  
By Attorneys

Aug. 3, 1937.

E. HUBERT ET AL

2,088,858

MANUFACTURE OF ARTIFICIAL THREADS

Filed April 30, 1935

3 Sheets-Sheet 3

Fig. 5



Fig. 6



Inventors:  
Emil Hubert  
Hans Dannerberg,  
Attorneys  
Potter, Peice & Scheffler.

By

## UNITED STATES PATENT OFFICE

2,088,858

## MANUFACTURE OF ARTIFICIAL THREADS

Emil Hubert, Dessau-Ziebigk, and Hans Dannenberg, Dessau, Germany, assignors to I. G. Farbenindustrie Aktiengesellschaft, Frankfort-on-the-Main, Germany

Application April 30, 1935, Serial No. 19,106  
In Germany March 9, 1933

2 Claims. (Cl. 18—54)

Our present invention relates to the art of manufacturing artificial threads.

It is a continuation-in-part of our co-pending application Ser. No. 714,721, filed March 8, 1934.

5 One of its objects is to provide a new process of manufacturing artificial silk and more particularly to a new process of assembling spun threads to an efficient package or cake for further treatment. Another object is the package 5 of threads obtained by our new process. Further objects will be seen from the detailed specification following hereafter. Reference is made to the accompanying drawings in which:

10 Figs. 1 and 1a illustrate the spinning process, Figs. 2, 3 and 4 show the manner in which the thread is deposited, and

15 Figs. 5 and 6 show conventional views of a finished package or cake.

It is known to produce artificial silk by causing 20 a thread spun in the usual way into a spinning bath and drawn off by a roller rotating at the required speed of draft to fall freely into a slowly rotating box in which the threads are collected.

25 In this process a regular deposition of the thread within the box is realized by imparting to the box a revolving and a reciprocating movement. In this manner the threads are piled cross-wise in the form of loose loops, which, when the box is filled, are reeled off from the box to 30 form hanks which may be after-treated in this form.

As artificial silk, in many cases, is no longer delivered to the consumer by the manufacturer 35 in the form of hanks, but in a wound form, it is no longer desirable to after-treat artificial silk in hank-form. The actual state of art, for avoiding any superfluous operation, requires the filaments to be after-treated in the form in which they were spun. This is not possible with the 40 loose layers of threads, such as they are produced in slowly rotating spinning pots as described. The loose layers suffer so much relative displacement by the washing and after-treating liquids that reeling off the content of 45 the spinning pot becomes impossible in most cases. In many cases the threads are rendered highly unfit for winding.

According to this invention we have found that it is possible to pile up the spun thread in form 50 of a solid cake capable of retaining its form in

handling it in the washing and after-treatment operations and which needs no support at all neither during its production nor in handling it as aforesaid. The cake produced in this manner may be washed and after-treated in the same 5 way as a centrifugal cake, while freely lying on a plate, or hanging on rods or arranged in any suitable manner, without incurring displacement of the threads or impairing their capacity of being wound. 10

The improvement is attained in the following way:

Referring to Fig. 1, the thread 1 issuing from the nozzle 2 and coagulated in the spinning bath 3 is guided around the roller 4 and the thread 15 falls from the roller 4 on the plate 5, which performs a rotary movement and an additional movement, for instance a reciprocating or an eccentric movement. The ratio between the period of the rotary movement and the period of 20 the additional movement must be so adjusted that the layers of threads deposited on the plate form a regular system of crossings in which each thread has its determined position. It is particularly advantageous to wind the threads in 25 such a manner that the windings lie closely side by side at a distance of about 2 to 5 mm. from each other. Fig. 3 shows the form of the windings which are deposited closely to each other and are helically piled up to form the cake. 30 Under these conditions the layers of thread form a body occupying a minimum of space and the cake being therefore very solid. In other words, the package of threads conserving its form in the usual treatment with liquid is obtained according to the present invention by a method of 35 winding the threads so as to save space. Fig. 4 shows for instance, diagrammatically the crossing of the thread in one layer. This figure has been obtained by covering with a paper a rotating plate to which an additional reciprocating movement has been imparted by a planetary gear and pressing a writing device, for instance, a pencil against the paper. 40

In order to obtain a completely unobjectionable 45 package of threads two further conditions must be considered. The first condition is that the additional movement of the plate must not be too quick. Preferably the additional movement corresponds approximately with two revolutions of 50

the plate that is to say one reciprocation must occur on somewhat more or less than two revolutions of the plate in which case the thread is deposited on the plate in double loops as shown in Fig. 2. If one reciprocation would occur on exactly one revolution or a whole number of revolutions an unserviceable cake or no cake at all is formed because in this case all loops would be deposited at the same place. The highest admissible speed is that at which one reciprocating movement takes place on every half turn of the plate. If the reciprocating additional movement is slower than the speed of the plate the thread is deposited on the plate in form of loops having a curvature which always appears concave when viewed from the center of the cake. If the reciprocating additional movement is quicker there are formed loops having varying curvature in such a manner that the curvature of the loops when viewed from the center of the cake alternately appears convex and concave. This form of loop is not favorable and yields unserviceable cakes when the reciprocating movement is quicker than the above mentioned limit of more than one reciprocation on half a revolution. A too quick reciprocating movement involves the further difficulty that the thread is no longer capable to follow the movement of the support with the required accuracy; in this case the thread comes not to lie at the intended place so that only a loose accumulation of threads occurs.

The second condition which must be considered for the production of an unobjectionable package of threads, is to stabilize the pendulum swingings which invariably occurs at the freely hanging part of the thread. The cause for this swinging will now be explained with reference to Fig. 2. The freely hanging thread is received by the plate 5 at 6, the speed of the thread being equal to the peripheral speed of point 6. However, by the additional movement the thread is guided alternately outwards, towards the path of point 7, and inwards, towards the path of point 8. Points 7 and 8 however, run at a higher and a lower speed than point 6. The thread, therefore, falls on a support which is moved alternately more swiftly and more slowly than the constant speed, at which the thread is supplied and, therefore, the thread is alternately pulled along or pushed back. The hanging thread, therefore, does not move on the path between the points 7 and 8, but, for instance, on the path between the points 9 and 10. Therefore the thread performs considerable pendulum swingings about the point 11 (see Fig. 1) at which the thread leaves the roller. In consequence the additional movement is the cause of these pendulum swingings.

As it has been found these pendulum swingings cause troubles only when taking an irregular course. In this case the winding system becomes less accurate. Furthermore, the thread easily forms small loops or knots or is deposited across the packages at its points of reversion. Completely uniform oscillations, however, do not interfere with the accuracy of the windings. The production of such uniform oscillations was realized by profiting of the resonance phenomena, which as is known occurs with any kind of oscillation. The free part of the thread which oscillates has a natural oscillation which depends on the weight of the thread, on the weight of the portions of the spinning bath adhering to the thread and on its dimensions. If the time of the natural oscillation corresponds with the period

of the additional movement of the rotating plate that is with the time of one reciprocation, resonance between the two is produced that is to say the thread oscillates uniformly and quickly without trembling or shaking and the formation of a regularly wound and solid cake occurs. Resonance is also produced if the time of oscillation and the time of revolution are in a ratio of 1:2, 1:3, 2:1, etc., that is to say in the case of a so-called harmonic. 10

The adjustment of the apparatus to produce resonance is very simple in practice. With a given titer and a given number of revolutions the distance between the galette and the rotary plate is varied until the oscillations have become 15 stable, a fact which may be recognized without difficulty because in this case the thread shows neither trembling nor shaking. For making slight corrections, it suffices to shift the point 11 in Fig. 1, at which the thread leaves the guide 20 roller, in lateral direction.

The mechanism preferably adopted in the process according to the present invention for imparting to the spinning box both a reciprocating and a rotary movement about its shaft is the 25 planetary gear described in our co-pending application Ser. No. 714,720, filed March 8, 1934. However, on principle, any device for executing a rotary movement and an additional reciprocating movement subject to the above condition is 30 suitable for use with the rotary plate for depositing threads.

The process of producing artificial silk according to this invention involves furthermore the 35 advantage that the spinning speed can be raised to 90 meters per minute up to 120 meters and even more.

If spinning is conducted at a high rate with the customary spinning baths and the thread is collected with cross-winding on a bobbin or in 40 a centrifugal box in known manner, it is found that the uniformity of the artificial silk thus made is unsatisfactory, this being particularly evident in that the fibres are dyed very unevenly. Variations in the composition of the spinning 45 bath or in the length of travel of the thread through the bath or in both do not suffice to provide a uniform artificial silk, particularly one which is capable of being dyed evenly and is suitable for working into fabrics. 50

It has been found that the cause of this lack of uniformity is to be found in the reciprocatory device which usually serves for laying the freshly spun thread in cross-wound layers on the bobbin or in the centrifugal box, in order that it may be 55 subjected to an after-treatment with liquids. The reciprocatory device moves the thread backwards and forwards with the aid of a thread-guide (an eye, back or spinning funnel), whereby it is impossible to avoid subjecting the thread to 60 jerks. At low and moderate spinning speeds these jerks remain within endurable limits but they increase very rapidly at higher speeds of spinning (about 90 meters per minute) and then give rise to the aforesaid lack of uniformity. 65

It may also be mentioned that spinning machines having a reciprocatory device naturally run less smoothly when they are operated at spinning speeds above 90 meters per minute; the oscillations thus caused are likewise communicated to the silk and influence the uniformity of the final product. 70

In accordance with the present invention it is possible to produce artificial silk which does not suffer from the aforesaid objection even with a 75

spinning speed exceeding 90 meters per minute, if the thread, after it has been coagulated in a suitable manner, is led to the winding device without the assistance of a thread-guide or spinning funnel. For this purpose there may be used as the winding device a support having the form of a plate, which executes a combined rotary and reciprocatory motion. This support is actuated most advantageously by means of a planetary drive. The thread which falls freely from a roller on to the support is caused by the rhythmic movement of the latter to execute pendulous oscillation, which replace the action of the reciprocating thread-guide and cause the deposition of the thread in cross-wound layers.

This manner of collecting the thread in high-speed spinning has proved to offer particular advantages, since the faults caused by the reciprocating thread-guide are thereby completely avoided. While in the known spinning processes the difficulties increase very rapidly with an increasing speed of spinning, it is surprising that the process of the invention has been found to operate at a spinning velocity of 120 meters per minute even better than at, for instance, 80 meters per minute; for the pendulous oscillations have at the higher spinning velocity a smaller amplitude owing to the formation of harmonics. In this manner there can be produced, even with very high speeds of draught, an artificial silk of unobjectionable quality in well formed durable windings.

In carrying out the process it has been found advantageous to use a spinning bath having a rapid coagulating action. It is to be recommended that in carrying out the process there should be used a spinning bath containing besides sulfuric acid and sodium sulfate a salt of a polyvalent metal, for example, zinc sulfate, magnesium sulfate or aluminium sulfate.

The following examples illustrate the invention:

#### Example 1

For a viscose thread with a titer of 180 den. prepared in a spinning bath having a specific weight of 1.4 and spun at a speed of 60 m. per minute, the resonance effect is obtained by giving the measures  $a$ ,  $b$ ,  $c$ ,  $d$  of Figs. 1 and 1a the following values:

$$\begin{aligned} a &= 725 \text{ mm.} \\ b &= 95 \text{ mm.} \\ c &= 80 \text{ mm.} \\ d &= 50 \text{ mm.} \end{aligned}$$

the cake obtained after 6 hours' spinning had the following dimensions:

| Thread package | Freshly spun acid moist | Washed and dried |
|----------------|-------------------------|------------------|
| Outer diameter | 190 mm.                 | 178 mm.          |
| Inner diameter | 100 mm.                 | 78 mm.           |
| Middle height  | 92 mm.                  | 51 mm.           |
| Weight         | 1,270 grams.            | 400 grams.       |
| Density        | 0.723 gram/cc.          | 0.360 gram/cc.   |

|                  |               |
|------------------|---------------|
| Total titer      | 180 deniers   |
| Single titer     | 5 deniers     |
| Length of thread | 20,000 meters |

#### Example 2

When spinning a viscose thread having a titer of 300 deniers at the same speed in a spinning

bath of the same specific weight the values of  $a$ ,  $b$ ,  $c$  and  $d$  are the following:

$$\begin{aligned} a &= 780 \text{ mm.} \\ b &= 150 \text{ mm.} \\ c &= 70 \text{ mm.} \\ d &= 50 \text{ mm.} \end{aligned}$$

the cake obtained after 6 hours' spinning had the following dimensions:

| Thread package      | Freshly spun acid moist | Washed and dried |
|---------------------|-------------------------|------------------|
| Outer circumference | 660 mm.                 | 625 mm.          |
| Outer diameter      | 210 mm.                 | 198 mm.          |
| Inner circumference | 375 mm.                 | 277 mm.          |
| Inner diameter      | 120 mm.                 | 88 mm.           |
| Middle height       | 135 mm.                 | 75 mm.           |
| Volume              | 3,150 cc.               | 1,853 cc.        |
| Weight              | 2,250 grams.            | 660 grams.       |
| Density             | 0.715 gram/cc.          | 0.356 gram/cc.   |

.5

10

20

|                      |               |
|----------------------|---------------|
| Total titer          | 300 deniers   |
| Single titer         | 5 deniers     |
| Length of the thread | 20,000 meters |

#### Example 3

Spinning solution Viscose containing 7-8 per cent of cellulose and 6-7 per cent of sodium hydroxide

30

Spinning bath 13 per cent of sulfuric acid, 18 per cent of sodium sulfate and 10 per cent of magnesium sulfate

35

Titer 180/36

Draught 120 meters per minute

Travel of thread in precipitating bath 70 centimeters

40

Device for removing 2 glass rods of 5 mm. diameter at distances of 10 and 30 mm. from threads above the surface of the bath

45

Device for collecting Plate actuated by planetary drive threads

Speed of rotation of the 224.6 R. P. M. plate

50

Planetary motion of the 110 R. P. M. plate

55

Distance of the middle point of the roller from the surface of the plate

Lateral displacement of 60 mm. backwardly and 300 mm. sideways the point at which the thread leaves the roller with respect to the axis of the planetary drive

65

Nature of pendulous The freely hanging oscillation. length of thread executes an oscillation showing two nodes

70

Figs. 5 and 6 show a finished cake. As seen from these figures in practice the inner and the outer border of the cake may show a slight deformation. The outer, upper edge of the cake is generally somewhat rounded whereas the inner,

75

upper border may be somewhat raised. The walls of the cake are perfectly smooth and vertical on the plate.

The diameter of the cake is determined by the speed at which the plate is rotated and the speed at which the thread is supplied. The mean diameter of the cake (see the dotted line in Fig. 2) is equal to

$$10 \quad \frac{\text{speed at which the thread is supplied}}{\pi \text{ number of revolutions of the plate}}$$

The breadth of the cake is approximately equal to the width of the reciprocating movement. The density of the dry cake may vary between 0.2 to 15 0.5 gram/cc. as has been found without however limiting our invention to these values.

According to our invention, there may be produced packages having a very great length of thread of about 20,000 meters or 30,000 meters 20 which varies with the titer of the spun thread. The advantage of the present invention over the hitherto used bobbin spinning system and centrifugal spinning results from the following table:

| 25 | Bobbin spinning           | Centrifugal spinning       | Plate spinning             |
|----|---------------------------|----------------------------|----------------------------|
|    | 100 grams<br>6,000 meters | 165 grams<br>10,000 meters | 500 grams<br>30,000 meters |

30 which is drafted for a titer of 150 deniers.

The process according to this invention obviously is not limited to spinning viscose silk as shown in the examples but is adapted for spinning spinning solutions according to the wet spinning process quite generally. Thus, there 35 may be spun solutions of cellulose acetate or another cellulose derivative or there may be spun solutions of fibroin according to the wet spinning process.

What we claim is:

1. A process of producing artificial silk which comprises ejecting a spinning solution into a precipitating bath, guiding the coagulated thread around a rotating roller, rotating said roller at a peripheral speed of at least 90 meters per minute, causing the thread to fall on a plate, rotating said plate at a speed so that a point of the plate at a substantial distance from the center of rotation has the same peripheral velocity as said roller, giving the plate an additional reciprocating movement so that at most one reciprocation occurs on half a revolution of the plate and adjusting the free length of the thread between the point at which the thread leaves the roller and the point at which the thread falls on the rotating plate so that the natural vibrations of the thread are in resonance with the reciprocating movement and a cake which needs no support is formed. 15

2. A process of producing artificial silk which comprises ejecting a spinning solution into a precipitating bath, guiding the coagulated thread around a rotating roller, rotating said roller at a peripheral speed of 120 mms. per minute, causing the thread to fall on a plate, rotating said plate 20 at 224.6 revolutions per minute, giving the plate an additional planetary motion of 110 revolutions per minute and adjusting the distance of the middle-point of the roller from the surface of the plate to 800 mms., adjusting the reciprocatory 25 movement to a width of 50 mms., adjusting the lateral displacement of the point at which the thread leaves the roller with respect to the axis of the planetary drive 60 mms. backwardly and 300 mms. sideways, and adjusting the supplied quantity of viscose to a final titer of 180 30 deniers.

EMIL HUBERT.  
HANS DANNENBERG.